

# United States Patent

[11] 3,615,488

[72] Inventors **Frank J. Drago;**  
Clinton Van Grol, both of Rochester, N.Y.  
[21] Appl. No. **20,791**  
[22] Filed **Mar. 18, 1970**  
[45] Patented **Oct. 26, 1971**  
[73] Assignee **Eastman Kodak Company**  
Rochester, N.Y.

[54] **PHOTOGRAPHIC PROCESSING COMPOSITION  
AND PROCESS COMPRISING CYSTEINE AND AN  
ALDEHYDE BISULFITE**  
26 Claims, No Drawings

[52] U.S. Cl..... **96/50,**  
96/66, 96/66.3  
[51] Int. Cl..... **G03c 5/26,**  
G03c 5/30  
[50] Field of Search..... **96/66.3,**  
66.5, 66, 50, 95

[56]

## References Cited

UNITED STATES PATENTS  
2,124,159 7/1938 Weyde ..... 96/61  
2,902,367 9/1959 Welliver et al. ..... 96/66.4  
3,128,180 4/1964 Henn et al. ..... 96/66.4

*Primary Examiner*—Norman G. Torchin

*Assistant Examiner*—Mary F. Kelley

*Attorneys*—Bernard D. Wiese, W. H. J. Kline and Myron B. Kurtzman

**ABSTRACT:** Photographic-processing composition for developing photographic elements in the presence of a developing agent such as hydroquinone, comprising cysteine, an aldehyde bisulfite such as sodium formaldehyde bisulfite and an organic antifoggant. The composition is advantageously employed in a continuous transport processing machine.

PHOTOGRAPHIC PROCESSING COMPOSITION AND  
PROCESS COMPRISING CYSTEINE AND AN ALDEHYDE  
BISULFITE

BACKGROUND OF THE INVENTION

1. FIELD OF THE INVENTION

This invention relates to photographic materials and their use. In one aspect, this invention relates to compositions employed in the development of high-contrast photographic elements. In another aspect, this invention relates to the process of developing exposed high-contrast photographic elements in a continuous transport processing machine wherein at least one processing solution comprises new photographic developer compositions.

2. DESCRIPTION OF THE PRIOR ART

In the graphic arts field, where it is desired to make photographic line and halftone reproductions, it is customary to employ emulsions having extremely high contrast. In development, the developing areas grow autocatalytically at a very high developing rate to produce an extremely high contrast. Developers for use with extremely high-contrast photographic films are quite different in composition from typical black-and-white film developers. In order to obtain very high contrast and sharp lines, it has been a practice to formulate developers for such films from essentially hydroquinone, an alkali, an alkali metal bromide and a low level of sulfite ion. The low level of sulfite ion partially stabilizes the developer solution for a short period of time and is achieved in all known commercial developers of this type by the use of an aldehyde sulfite, such as sodium formaldehyde bisulfite, which acts as a sulfite ion buffer. These developer solutions are generally stored in two parts since, for example, the sodium formaldehyde bisulfite will dissociate at a high pH to give not only the desired sulfite ion but an equimolar amount of formaldehyde which will react with hydroquinone to destroy the developing power.

The developer solutions for high-contrast films presently used in continuous transport processing machines have a number of disadvantages. For example, all of the prior lith-developers have a relatively low capacity and begin to show substantial exhaustion after the development of a relatively small amount of lith-film and solution either discarded in commercial practice or replenished. It is also well known that the aldehyde bisulfites such as sodium formaldehyde bisulfite may cause some loss in speed, but more importantly may cause a loss in Dmax of the developed image. While the prior art has disclosed good high contrast images for normal conditions of time and temperature, it is of particular concern to improve the negative density and decrease line veiling in fast access processing at high temperatures in automatic processing equipment, such as the Kodak Supermatic Processor. It would be very desirable to have a developer solution for high-contrast films which could be used in high temperature continuous transport processing machines without obtaining line veiling, while at the same time obtaining a higher capacity in machine or tray processing for such a developer solution.

In many instances it is advantageous to process high-contrast films by means of an activator solution, if the developing agent is incorporated in the light-sensitive element. Such an activation process is particularly desirable to provide longer tray life of processing solution since an alkali processing solution without a developing agent will be less subject to auto-oxidation. Suitable incorporated developer emulsions have been described in French Pat. No. 1,479,090. Typical emulsion compositions would comprise a silver chlorobromide gelatin emulsion (80 mole percent chloride) containing hydroquinone and coated on a polyester film support to yield the following coverages: Silver 410 mg. per square foot, gelatin 900 mg. per square foot and hydroquinone 150 mg. per square foot. If desired, part of the gelatin may be replaced with a synthetic vinyl polymer such as an alkyl-acrylate latex. Our invention is advantageously carried out with alkaline activator solutions which do not contain any developing agent or less developing agent than is required for full development activity.

SUMMARY OF THE INVENTION

In accordance with this invention, there is provided a novel and unobvious high-contrast processing solution which manifests an increase life and capacity while at the same time producing negatives of very good image tone and image sharpness. The improvements of the present invention are obtained by employing a processing solution comprising cysteine and a monoaldehyde which work synergistically to produce the desired effects.

It is therefore an object of the present invention to provide a new high-contrast processing solution. A further object is to provide a new high-contrast developer solution which has improved keeping properties and also improved solution life in terms of aeration and film capacity. It is still a further object to provide a high-contrast developer solution which produces developed images showing a high Dmax, improved tone, good image sharpness and improved edge effects. Another object of the invention is to provide an alkaline processing solution for the development of lith-type silver halide films which have therein one or several of a variety of silver halide developing agents. Other objects of this invention will become obvious to those skilled in the art from that which appears hereinafter.

25 DESCRIPTION OF THE PREFERRED EMBODIMENTS

According to an embodiment of this invention, there is provided an essentially bromide-free, high contrast processing solution containing a monoaldehyde and cysteine in the presence of a silver halide developing agent which exhibits the unexpected and unobvious properties referred to above. In the preferred embodiments of the invention, the developer solution additionally contains an organic antifoggant.

According to another embodiment of this invention, there is provided an essentially bromide-free, high-contrast activator solution containing a monoaldehyde and cysteine for the processing of a photographic elements having a developing agent incorporated therein.

The monoaldehyde bisulfites which can be employed in the novel developer compositions are desirably alkali metal, lower hydrocarbyl and desirably lower aliphatic, monoaldehyde bisulfites. The monoaldehyde bisulfites are well known as shown by Donovan et al. U.S. Pat. No. 2,313,523 issued Mar. 9, 1943, and Kridel et al. U.S. Pat. No. 2,843,483 issued July 15, 1958. Illustrative of the aldehydes bisulfites which may be advantageously employed are sodium formaldehyde bisulfite, potassium formaldehyde bisulfite, sodium acetaldehyde bisulfite and sodium isobutyraldehyde bisulfite. A preferred monoaldehyde bisulfite is sodium formaldehyde bisulfite. The concentration of the aldehyde bisulfite suitably employed in our developer composition is from about 0.05 to about 1.0 moles per liter of developer composition and is preferably about 0.3 moles per liter of developer composition.

The developing agents, which can be employed in our developing solutions can be any of those commonly employed in the graphic arts. Useful silver halide developing agents, for example, include dihydroxy benzenes such as hydroquinone; chlorohydroquinone; bromohydroquinone; 2,3-dichlorohydroquinone; 2,5-dimethylhydroquinone; 2,3-dibromohydroquinone; 1,4-dihydroxy-2-acetophenone-2,5-dimethylhydroquinone; 2,5-diethylhydroquinone; 2,5-di-p-phenethylhydroquinone; 2,5-dibenzoylaminohydroquinone; 2,5-diacetaminohydroquinone; etc. [Esters of such compounds, for example, formates and acetates can also be employed.] These developing agents can be used alone or in any combination and can be employed in any concentration which is effective for development. A suitable concentration for the developing agent is about 0.05 to about 0.50 mole per liter of developing composition and is typically from 0.10 to about 0.03 mole per liter of developer composition.

The cysteine in our novel processing composition is L-cysteine ( $\beta$ -mercaptoalanine). As will be understood hereinafter, the use of the term cysteine will include not only the amino acid but also its hydrohalides. Suitable concentra-

tions of the cysteine are from about 0.1 to about 0.9 grams per liter of developer composition and preferably about 0.3 grams per liter of developer composition.

Our novel processing compositions generally do not employ bromides as restrainers. In place of the bromide restrainers, we employ organic antifoggants. Should bromide, for example, potassium bromides which is normally employed in lith developer solutions, be utilized, the improved image tone and improved developer activity, the higher line density, and the improved solution life obtained are minimized. The organic antifoggants are well known as discussed, for instance, in Mees, *The Theory of the Photographic Process*, 3rd Edition, (1966), p. 344-346. In a preferred embodiment of this invention the organic antifoggants can be benzimidazoles or indazoles. In another preferred embodiment of this invention, the organic antifoggants can be the nitrobenzimidazoles and nitroindazoles. Illustrative of the organic antifoggants which can be employed in our developer solutions are: 5-nitrobenzimidazole, 5-nitroindazole and 6-nitrobenzimidazole nitrate.

Suitable concentrations for the organic antifoggants range from about 0.1 to about 2.0 grams per liter of developer composition and preferably about 0.8 grams per liter of developer composition for fast access high temperature processing. About one half these amounts are suitable for normal temperature (68° F.) tray processing. The preferably organic antifoggants are the nitrosubstituted organic antifoggants.

Optimum results are obtained when employing our processing composition by maintaining the pH of the solution between about 10 and about 11.2. When machine processing, for example, in a machine such as Kodak Supermatic Processor Model 242 optimum results are obtained by maintaining the temperature of the processing solutions between about 90° F. and 130° F. and preferably about 110° F. When tray processing, the temperature can range from about 60 to 80° F.

Our novel processing composition and activator solutions can be utilized either in tray processing or preferably in a continuous machine processing system, such as the fast access high-temperature transport machines, wherein the high-contrast photographic element is processed by passing through rollers or otherwise in one continuous motion by transporting it into and out of at least one processing solution in the manner shown, for example, by U.S. Pats. Nos. 3,025,779 of Russell and Kunz issued Mar. 20, 1962; 3,078,024 of Sandeson issued Feb. 19, 1963; 3,122,086 of Fitch issued Feb. 25, 1964; 3,149,551 of Cramer issued Feb. 22, 1964; 3,156,173 of Meyer issued Nov. 10, 1964; and 3,224,356 of Fleisher and Hixon issued Feb. 21, 1965. The continuous transport process may be described as a "unidirectional" transport process. By the term unidirectional it is understood that the photographic elements move over all in one direction; however, the general movement would include up and down movements, etc. to accommodate rollers, processing solutions, etc.

This invention can be further illustrated by the following examples of preferred embodiments thereof, although it will be understood that these examples are included merely for illustrating this invention.

#### EXAMPLE I

Sheets of a high contrast chlorobromide emulsion are sensitometrically exposed to a 0.01 density step tablet. Individual sheets are developed respectively in one of developer solutions A, B, C, or D in a Kodak Supermatic Processor at 110° F. A. Developer Composition without Cysteine and Sodium Formaldehyde Bisulfite

|                                          |            |
|------------------------------------------|------------|
| Hydroquinone                             | 33.0 grams |
| 5-nitrobenzimidazole nitrate             | 1.1 grams  |
| Triethylene glycol                       | 60.0 ml.   |
| Sodium bicarbonate                       | 70.0 grams |
| Potassium hydroxide                      | 47.0 grams |
| Sodium sulfite                           | 8.0 grams  |
| Trisodium phosphate (12H <sub>2</sub> O) | 16.0 grams |
| Aminoethanol                             | 4.0 grams  |
| Water to make                            | 1.0 liter  |

pH adjusted to 10.6

#### B. Developer Composition

Developer Composition A+40 grams of Sodium Formaldehyde Bisulfite.

#### C. Developer Composition of the Invention

Developed Composition A+40 grams Sodium Formaldehyde Bisulfite and 0.3 grams cysteine.

#### D. Developer Composition A+0.3 grams cysteine.

10 The results of processing the exposed films are summarized in table I.

TABLE I

| Developer | Relative Speed Log E | Gamma | Effective Contrast (Toe Contrast) |                  | D <sub>min</sub> | D <sub>max</sub> | Solution <sup>2</sup> Life |
|-----------|----------------------|-------|-----------------------------------|------------------|------------------|------------------|----------------------------|
|           |                      |       | D <sub>min</sub>                  | D <sub>max</sub> |                  |                  |                            |
| A         | .00                  | 5.5   | 3.7                               | 0.04             | 5.2              | <1 Hr.           |                            |
| B         | -.05                 | 4.5   | 4.0                               | 0.05             | 4.7              | 1 Hr.            |                            |
| C         | +.05                 | 5.0   | 4.0                               | 0.04             | 5.7              | 2 Hr.            |                            |
| D         | .00                  | 4.0   | 1.8                               | 0.11             | 5.2              | <1 Hr.           |                            |

<sup>2</sup> One gallon is circulated at 110° F in Kodak Supermatic Processor Model 242 (1 hr of solution life equals 12 hrs machine life when 5 gallons of developer are used).

25

The above data show that the developer composition B absent cysteine shows a slight loss in speed, a significant loss in D<sub>max</sub> and also has a low solution life. Developer solution containing both sodium formaldehyde bisulfite and cysteine provides a speed increase, a significant increase in D<sub>max</sub> and the solution life is doubled.

30 A developer solution identical to Developer A but also containing 0.3 grams cysteine (Developer D) causes a significant decrease in toe contrast and an undesirable increase in fog.

#### EXAMPLE II

40 This example illustrates the excellent capacity of the developer solutions of the invention. A developer solution is prepared having the following formulations:

|                                        |             |
|----------------------------------------|-------------|
| Sodium formaldehyde bisulfite (Pract.) | 50 Grams    |
| Sodium carbonate (monohydrate)         | 60 Grams    |
| Potassium carbonate (anhydrous)        | 60 Grams    |
| Sodium phosphate (tribasic crystal)    | 21.5 Grams  |
| Sodium sulfite (anhydrous)             | 10.8 Grams  |
| 6-nitrobenzimidazole nitrate           | 1.125 Grams |
| Hydroquinone                           | 33 Grams    |
| L-cysteine, free base                  | 00.43 Grams |
| Tri-ethylene glycol                    | 50.6 Grams  |
| 2-aminoethanol                         | 10 Grams    |
| Water to make                          | 1.0 Liter   |

55 Sheets of a high-contrast chlorobromide emulsion are sensitometrically exposed to a 0.10 step tablet and processed at a rate of 2½f.p.m. at 110° F. in a Kodak Supermatic Processor. The results of the tests as to capacity are summarized in table II.

60

TABLE II

| Exhaustion <sup>1</sup> Rate | Relative Log Speed | γ   | D <sub>max</sub> | D <sub>min</sub> | Line Negative Quality |
|------------------------------|--------------------|-----|------------------|------------------|-----------------------|
| Fresh                        | 5.90               | 6.0 | 3.9              | 0.07             | Good Excellent        |
| 350 Ft. <sup>2</sup>         | 5.85               | 5.0 | 3.7              | 0.07             | Good Excellent        |
| 700 Ft. <sup>2</sup>         | 5.90               | 6.0 | 3.6              | 0.06             | Excellent             |
| 1050 ft. <sup>2</sup>        | 5.85               | 6.5 | 3.5              | 0.05             | Excellent             |

70 <sup>1</sup> Per 5 gallon container.

#### EXAMPLE III

75 A developer composition (A) identical to that in example II is prepared. A similar solution (B) is prepared except cysteine.

Strips of a high-contrast chlorobromide emulsion are exposed to a 0.1 density step tablet and tray processed to simulate machine conditions at 110° F. in the developer solutions. The results of the sensitometric tests are summarized in table III.

TABLE III

| Developer | Relative Log Speed | $\gamma$ | D <sub>max</sub> | D <sub>min</sub> |
|-----------|--------------------|----------|------------------|------------------|
| A         | 5.95               | 7.0      | 4.20             | 0.04             |
| B         | 5.60               | 6.1      | 3.35             | 0.04             |

## EXAMPLE IV

This example illustrates the exceptional capacity of our developer composition over prior art developer composition when employed in tray processing.

The high-contrast developer compositions are prepared as follows:

## A. Developer Composition Containing Cysteine and Sodium Formaldehyde Bisulfite

Sodium formaldehyde bisulfite (practical) 40 grams/l  
Sodium carbonate (monohydrate, granular) 60 grams/l  
Potassium carbonate (anhydrous) 60 grams/l  
Sodium phosphate (tribasic, crystal) 30 grams/l  
Sodium sulfite (anhydrous) 4 grams/15-Nitrobenzimidazole 0.26 grams/l  
5-Nitroindazole 0.04 grams/l  
Boric acid 3 grams/l  
Hydroquinone 20 grams/l  
L-Cysteine, free base (8 mercaptoalanine) 0.33 grams/l  
2,5-Dithiobiurea 0.10 grams/l  
Water to make 1.0 liter

## B. Prior Art ("Lith" Type Developers)

Sodium formaldehyde bisulfite 70 grams/l  
Hydroquinone 15 grams/l  
Sodium carbonate (monohydrate) 75 grams/l  
Potassium bromide 3 grams/l  
Water to make 1 liter

C. Prior Art (Copy Line Developer)

Sodium formaldehyde bisulfite 50 grams/l  
Hydroquinone 15 grams/l  
Sodium carbonate (monohydrate) 20 grams/l  
Potassium bromide 0.1 grams/l  
Water to make 1 liter

Test exposures of line reflection originals were made in a copy camera using 1,200 foot-candles incident illumination to produce line negatives on a high-contrast chlorobromide emulsion. The results of the capacity tests are summarized in table IV and the sensitometric tests are summarized in table V.

TABLE IV

| Developer | Processing Time (Minutes) | Temp.  | Capacity (8×10-inch shts/gal) |
|-----------|---------------------------|--------|-------------------------------|
| A         | 1*                        | 70° F. | 100                           |
| B         | 2½*                       | 70° F. | 32                            |
| C         | ¾*                        | 70° F. | 16                            |

\* Agitation

\*\* Still

TABLE V

| Developed In | Properties of Developer Image Line Negative Quality    | Image Tone  |
|--------------|--------------------------------------------------------|-------------|
| A            | Good-excellent—copies both fine and coarse lines       | Black       |
| B            | Fair-good—copies some fine lines, and all coarse lines | Brown-Black |
| C            | Good-excellent—copies both fine and coarse lines       | Brown       |

## EXAMPLE V

A suitable alkaline activator solution according to the in-

vention provides for excellent quality of developed images in high-contrast emulsions containing incorporated developing agent. Such activator solutions have excellent keeping and exhaustion characteristics when compared to developing solutions

5 containing reducing agents. Since problems with keeping are reduced, activator solutions may be prepared which have higher pH's which desirably shorten the processing time.

Further, such solutions may be used at elevated temperatures with less deterioration on keeping. An example of the use of 10 an activator solution of our invention at high temperature in machine processing is given below: A solution was prepared to contain:

|    |                               |           |
|----|-------------------------------|-----------|
| 15 | Sodium formaldehyde bisulfite | 40.0 g    |
|    | Sodium carbonate              | 60.0 g    |
|    | Potassium carbonate           | 60.0 g    |
|    | Sodium phosphate              | 30.0 g    |
|    | 5-Nitrobenzimidazole          | 1.2 g     |
|    | 5-Nitroindazole               | 0.45 g    |
|    | L-cysteine                    | 0.8 g     |
|    | 2,5-Dithiobiurea              |           |
|    | Water to make                 | 1.0 liter |
|    | pH about 11.8                 |           |

The activator was used in a Kodak Supermatic Processor to 25 process a high-contrast silver chlorobromide film containing incorporated hydroquinone developing agent. The processing was carried out at 110° F. at 3 f.p.m. The activator solution was used for processing sheets of film containing typical negatives having at least 85 percent of the area exposed. Very good 30 results were obtained with the activator, even after 1,000 square feet of film had been processed in only 5 gallons of the activator. Data below show the sensitometric results on sheets of film after various amounts of film were processed.

| Exhaustion Rate          | Relative Speed | D <sub>max</sub> | D <sub>min</sub> | Quality   |
|--------------------------|----------------|------------------|------------------|-----------|
| 3.5 Fresh                | 0              | 3.8              | 0.05             | Excellent |
| 200 ft <sup>2</sup>      | 0              | 3.6              | 0.05             | Excellent |
| 400 ft <sup>2</sup>      | -0.05          | 3.5              | 0.05             | Excellent |
| 600 ft <sup>2</sup>      | -0.05          | 3.6              | 0.05             | Excellent |
| 800 ft <sup>2</sup>      | -0.10          | 3.4              | 0.05             | Excellent |
| 40 1,000 ft <sup>2</sup> | -0.10          | 3.4              | 0.05             | Very Good |

The results illustrate the excellent exhaustion characteristics of the activator. The exhaustion characteristics are obtained with very little change in speed and only minor change in D<sub>max</sub>.

## EXAMPLE VI

A suitable activator solution for tray processing at room temperature of an incorporated developer lith emulsion may 50 be prepared as follows:

|    |                                |         |
|----|--------------------------------|---------|
| 55 | Sodium formaldehyde bisulfite  | 20.00 g |
|    | Sodium carbonate (monohydrate) | 30.00 g |
|    | Potassium carbonate anhydrous  | 30.00 g |
|    | Sodium phosphate tribasic      | 15.00 g |
|    | 5-Nitrobenzimidazole           | 0.14 g  |
|    | 5-Nitroindazole                | 0.14 g  |
|    | L-Cysteine                     | 0.40 g  |
|    | 2,5-Dithiobiurea               | 0.10 g  |
|    | pH adjusted to 11.4            |         |

60 Sheets of exposed lith film comprising a high contrast chlorobromide emulsion containing norbornene hydroquinone developing agent were processed for 30 seconds at 68° F. in shallow trays containing the above solution. Excellent quality and density resulted. When a comparison test was run using 65 a similar activator from which the cysteine had been eliminated, lower densities and poorer line quality resulted.

Activator solution according to our invention may be prepared as a working solution or in more concentrated form as a liquid within the solubility limits of the chemicals involved. Successful concentrations have been prepared for 1:3 dilution with water.

The high-contrast emulsion processed with the processing 70 solutions of this invention may be unwashed or washed to remove soluble salts. In the latter case, the soluble salts may be removed by chill-setting and leaching or the emulsion may be coagulation washed, e.g. by the procedures described in

Hewitson et al. U.S. Pat. No. 2,618,556 issued Nov. 18, 1952; Yutzy et al. U.S. Pat. No. 2,614,928 issued Oct. 21, 1952; Yackel U.S. Pat. No. 2,565,418 issued Aug. 21, 1951; Hart et al. U.S. Pat. No. 3,241,969 issued Mar. 22, 1966 and Waller et al. U.S. Pat. No. 2,489,341 issued Nov. 29, 1949.

The emulsions processed with the processing solutions of this invention may be sensitized with chemical sensitizers, such as with reducing agents; sulfur, selenium or tellurium compounds; gold, platinum or palladium compounds; or combinations of these. Suitable procedures are described in Shepard et al. U.S. Pat. No. 1,623,499 issued Apr. 5, 1927; McVeigh U.S. Pat. No. 3,297,447 issued Jan. 10, 1967; Waller et al. U.S. Pat. No. 2,399,083 issued Apr. 23, 1946; and Dunn U.S. Pat. No. 3,297,446 issued Jan. 10, 1967.

The high-contrast emulsions and other hardenable layers processed in the processing solutions of this invention can be hardened by various organic or inorganic hardeners, alone or in combination, such as the aldehydes, and blocked aldehydes, ketones, carboxylic and carbonic acid derivatives, sulfonate esters sulfonyl halides and vinyl sulfonyl ethers, active halogen compounds, epoxy compounds, aziridines, active olefins, isocyanates, carbodiimides, mixed function hardeners and polymeric hardeners such as oxidized polysaccharides like dialdehyde starch and oxyguargum and the like.

The high-contrast emulsions and elements employed in the practice of this invention can contain various colloids alone or in combination as vehicles, binding agents and various layers. Suitable hydrophilic materials include both naturally occurring substances such as proteins, for example, gelatin, gelatin derivatives, cellulose derivatives, polysaccharides such as dextran, gum arabic and the like; and synthetic polymeric substances such as water soluble polyvinyl compounds like poly(vinylpyrrolidone), acrylamide polymers and the like.

The high-contrast emulsions and other layers of the high-contrast elements employed in the practice of this invention can also contain alone or in combination with hydrophilic, water permeable colloids, other synthetic polymeric compounds such as dispersed vinyl compounds such as in latex form and particularly those which increase the dimensional stability of the photographic materials. Suitable synthetic polymers include those described, for example, in Nottorf U.S. Pat. No. 3,142,568 issued July 29, 1964; White U.S. Pat. No. 3,193,386 issued July 6, 1965; Houck et al. U.S. Pat. No. 3,062,674 issued Nov. 6, 1962; Houck et al. U.S. Pat. No. 3,220,844 issued Nov. 30, 1965; Ream et al. U.S. Pat. No. 3,287,289 issued Nov. 22, 1966; Dykstra U.S. Pat. No. 3,411,911 issued Nov. 19, 1968; particularly effective are those water-insoluble polymers of alkyl acrylates and methacrylates, acrylic acid, sulfoalkyl acrylates or methacrylates, those which have cross-linking sites which facilitate hardening or curing, those having recurring sulfobetaine units as described in Dykstra Canadian Pat. No. 774,054.

The high-contrast elements processed in the presence of the novel processing solutions of this invention may contain anti-static or conducting layers, such layers may comprise soluble salts, e.g. chlorides, nitrates, etc., evaporated metal layers, ionic polymers such as those described in Minsk U.S. Pat. No. 2,861,056 issued Nov. 18, 1958, and Sterman et al. U.S. Pat. No. 3,206,312 issued Sept. 14, 1965, or insoluble inorganic salts such as those described in Trevoy U.S. Pat. No. 3,428,451 issued Feb. 18, 1969.

The high-contrast elements and other layers processed in the processing solutions of this invention can be coated on a wide variety of supports. Typical supports include cellulose nitrate film, cellulose ester film poly(vinyl acetal) film, polystyrene film, poly(ethylene terephthalate) film, polycarbonate film and related films or resinous materials, as well as glass, paper, metal and the like. Typically, a flexible support is employed, especially a paper support, which can be partially acetylated or coated with baryta and/or an alphaolefin polymer, particularly a polymer of an alpha-olefin containing two to ten carbon atoms such as polyethylene, polypropylene, ethylenebutene copolymers and the like.

The high-contrast elements and other layers processed in the processing solutions of this invention can contain plasticizers and lubricants such as polyalcohols, e.g. glycerin and diols of the type described in Milton et al. U.S. Pat. No. 2,960,404 issued Nov. 1, 1966; fatty acids or esters such as those described in Robijns U.S. Pat. No. 2,588,765 issued Mar. 11, 1952 and Duane U.S. Pat. No. 3,121,060 issued Feb. 11, 1964; and silicone resins such as those described in DuPont British Pat. No. 955,061.

10 The high-contrast elements and other layers employed in the practice of this invention may contain surfactants such as saponin; anionic compounds such as the alkyl aryl sulfonates described in Balsdiefen U.S. Pat. No. 2,600,831 issued June 17, 1962; amphoteric compounds such as those described in Ben-Ezra U.S. Pat. No. 3,133,816 issued May 19, 1964; and water soluble adducts of glycitol and an alkyl phenol such as those described in Olin Mathieson British Pat. No. 1,002,878.

15 The high-contrast elements and other layers employed in the practice of this invention may contain matting agents such as starch, titanium dioxide, zinc oxide, silica, polymeric beads including beads of the type described in Jelley et al. U.S. Pat. No. 2,992,101 issued July 11, 1961, and Lynn U.S. Pat. No. 2,701,245 issued Feb. 1, 1955.

20 The high-contrast elements and other layers employed in this invention may contain brightening agents including stilbenes, triazines, oxazoles and coumarin brightening agents. Water soluble brightening agents may be used such as those described in Albers et al. German Pat. No. 972,067 and McFall et al. U.S. Pat. No. 2,933,390 issued Apr. 19, 1960, or dispersions of brighteners may be used such as those described in Jansen German Pat. No. 1,150,274, Oetiker et al. U.S. Pat. No. 3,406,070 issued Oct. 15, 1968, and Heidke French Pat. No. 1,530,244.

25 The high-contrast elements and other layers employed in this invention may contain sensitizing agents including stilbenes, triazines, oxazoles and coumarin brightening agents. Water soluble brightening agents may be used such as those described in Albers et al. German Pat. No. 972,067 and McFall et al. U.S. Pat. No. 2,933,390 issued Apr. 19, 1960, or dispersions of brighteners may be used such as those described in Jansen German Pat. No. 1,150,274, Oetiker et al. U.S. Pat. No. 3,406,070 issued Oct. 15, 1968, and Heidke French Pat. No. 1,530,244.

30 40 45

Sensitizing dyes useful in sensitizing such emulsions are described, for example, in Brooker et al. U.S. Pat. No. 2,526,632 issued Oct. 24, 1950; Sprague U.S. Pat. No. 2,503,776 issued Apr. 11, 1950; Brooker et al. U.S. Pat. No. 2,493,748 issued Oct. 10, 1950; and Taber et al. U.S. Pat. No. 3,384,486 issued May 21, 1968. Spectral sensitizers which can be used include the cyanines, merocyanines, complex (tri- or tetrnuclear) merocyanines, complex (tri- or tetrnuclear) cyanines, holopolar cyanines, styryls, hemicyanines (e.g. enamine hemicyanines), oxonols and hemioxonols.

50 55 60 65

Dyes of the cyanine classes may contain such basic nuclei as the thiazolines, oxazolines, pyrrolines, pyridines, oxazoles, thiazoles, selenazoles and imidazoles. Such nuclei may contain alkyl, alkylene, hydroxyalkyl, sulfoalkyl, carboxyalkyl, aminoalkyl, and enamine groups and may be fused to carbocyclic or heterocyclic ring systems either unsubstituted or substituted with halogen, phenyl, alkyl, haloalkyl, cyano, or alkoxy groups. The dyes may be symmetrical or unsymmetrical and may contain alkyl, phenyl, enamine or heterocyclic substituents on the methine or polymethine chain.

70 75

The merocyanine dyes may contain the basic nuclei mentioned above as well as acid nuclei such as thiohydantoins, rhodanines, oxazolidenediones, thiazolidenedions, barbituric acids, thiazolineones, and malononitrile. These acid nuclei may be substituted with alkyl, alkylene, phenyl, carboxyalkyl, sulfoalkyl, hydroxyalkyl, alkoxyalkyl, alkylamino groups, or heterocyclic nuclei. Combinations of these dyes may be used, is desired. In addition, supersensitizing addenda which do not absorb visible light may be included, for instance, ascorbic acid derivatives, azaindenes, cadmium salts, and organic sul-

fonic acids as described in McFall et al. U.S. Pat. No. 2,933,390 issued Apr. 19, 1960, and Jones et al. U.S. Pat. No. 2,937,089 issued May 17, 1960.

The high-contrast elements and other layers processed in the processing solutions of this invention can contain light-absorbing materials and filter dyes such as those described in Sawdey U.S. Pat. No. 3,253,921 issued May 31, 1966, Gasper U.S. Pat. No. 2,274,782 issued Mar. 3, 1942; Silberstein et al. U.S. Pat. No. 2,527,583 issued Oct. 31, 1950; and VanCammen U.S. Pat. No. 2,956,879 issued Oct. 18, 1960. If desired, the dyes can be mordanted, for example, as described in Jones et al. U.S. Pat. No. 3,282,699 issued Nov. 1, 1966.

The invention has been described in detail with particular reference to preferred embodiments thereof, but it will be understood that variations and modifications can be effected within the spirit and scope of the invention.

I claim:

1. An essentially bromide-free photographic developer composition comprising:

- a. a silver halide developing agent,
- b. cysteine, and
- c. a monoaldehyde bisulfite.

2. The composition of claim 1 which additionally comprises an organic antifoggant.

3. The composition of claim 2, said composition being as aqueous solution.

4. The composition of claim 3 wherein said developing agent is present in a concentration of from about 0.05 to about 0.50 mole per liter of developer composition, said cysteine is present in a range of from about 0.1 to about 0.9 grams per liter of developer composition, said aldehyde bisulfite is present in a range of from about 0.05 to about 1.0 moles per liter of developer composition and said organic antifoggant is present in a range of from about 0.1 to about 2.0 grams per liter of developer composition.

5. The composition of claim 2 wherein said developing agent is a dihydroxybenzene developing agent and said monoaldehyde bisulfite is a formaldehyde bisulfite.

6. The composition of claim 5 wherein said dihydroxybenzene developing agent is hydroquinone, said formaldehyde bisulfite is sodium formaldehyde bisulfite and said organic antifoggant is a nitro-substituted organic antifoggant.

7. The composition of claim 6 wherein said nitrosubstituted organic antifoggant is one of 5-nitroindazole, 5-nitrobenzimidazole and 5-nitrobenzimidazole nitrate.

8. The composition of claim 1 wherein the pH is in a range of from about 10 to about 11.2 and additionally comprises free sulfite in the range of from about 2 to about 40 grams per liter of developer composition.

9. The composition of claim 6 wherein said hydroquinone is present in a concentration of about 0.3 mole per liter of developer composition, said cysteine is present in a concentration of about 0.003 mole per liter of developer composition, said sodium formaldehyde bisulfite is present in a concentration of about 0.3 mole per liter of developer composition and said organic antifoggant is present in a concentration of about 0.005 mole per liter of developer composition.

10. In a continuous unidirectional fast access high-temperature transport process for developing and processing an exposed, high-contrast photographic silver halide element, the improvement comprising developing said element in a liquid developer composition comprising:

- a. a silver halide developing agent,
- b. cysteine, and
- c. a monoaldehyde bisulfite.

11. In a continuous process of claim 10 wherein said developer composition additionally comprises an organic antifoggant.

12. In a continuous process of claim 11 wherein said developer composition is in the form of an aqueous solution.

13. In a continuous process of claim 12 wherein said developing agent is present in a range in a concentration of from about 0.05 to about 0.50 mole per liter of developer composition, said cysteine is present in a range of from about 0.1 to about 0.9 grams per liter of developer composition, said aldehyde bisulfite is present in a range of from about 0.05 to about 1.0 moles per liter of developer composition and said organic antifoggant is present in a range of from about 0.1 to about 2.0 grams per liter of developer composition.

14. In a continuous process of claim 13 wherein said developing agent is a dihydroxybenzene developing agent and said monoaldehyde bisulfite is a formaldehyde bisulfite.

15. In a process of claim 14 wherein said dihydroxybenzene developing agent is hydroquinone, said formaldehyde bisulfite is sodium formaldehyde bisulfite and said organic antifoggant is a nitro-substituted organic antifoggant.

16. The process of claim 15 wherein said nitrosubstituted organic antifoggant is one of 5-nitroindazole, 5-nitrobenzimidazole, 6-nitrobenzimidazole nitrate or 5-nitrobenzimidazole nitrate.

17. The process of claim 12 wherein said developing composition is at a pH of about 10 to about 11.2 and comprises from about 2 to about 40 grams per liter of a free sulfite.

18. The process of claim 10 wherein said photographic element comprises a silver halide emulsion in which the halide comprises at least 60 mole percent chloride.

19. The process of claim 15 wherein said hydroquinone is present in the concentration of about 0.3 mole per liter of developer composition, said cysteine is present in a concentration of about 0.003 mole per liter of developer composition, said sodium formaldehyde bisulfite is present in a concentration of about 0.3 mole per liter of developer composition and said organic antifoggant is present in a concentration of about 0.005 mole per liter of developer composition.

20. The process of claim 10 wherein said photographic element is transported by rollers.

21. In a process of processing an exposed, high-contrast photographic element, the improvement comprising developing said element in a liquid developer composition comprising:

- a. a silver halide developing agent,
- b. cysteine, and
- c. a monoaldehyde bisulfite.

22. The process of claim 21 where said developer composition additionally comprises an organic antifoggant and said monoaldehyde bisulfite is sodium formaldehyde bisulfite.

23. An essentially bromide-free alkaline photographic activator solution comprising a monoaldehyde bisulfite, cystine and at least one organic antifoggant.

24. An alkaline photographic activator solution of claim 23 wherein said organic antifoggant is nitrosubstituted and said monoaldehyde bisulfite is sodium formaldehyde bisulfite.

25. In a method of processing an exposed gelatino photographic silver halide element, said element containing a silver halide developing agent, the improvement comprising processing said element in the presence of an activator solution of claim 21.

26. In a method of processing an exposed gelatino photographic silver halide element, said element containing a silver halide developing agent, the improvement comprising processing said element in the presence of an activator solution of claim 24.